

# UNITED STATES PATENT OFFICE.

BENJAMIN F. DIMM, OF ERIE, PENNSYLVANIA, ASSIGNOR TO CHARLES A. DIMM,  
TRUSTEE.

## PROCESS OF ALLOYING ZINC WITH IRON OR STEEL.

1,307,853.

Specification of Letters Patent. Patented June 24, 1919.

No Drawing.

Application filed February 19, 1914. Serial No. 819,652.

To all whom it may concern:

Be it known that I, BENJAMIN F. DIMM, a citizen of the United States, residing at Erie, in the county of Erie and State of Pennsylvania, have invented new and useful Improvements in Processes of Alloying Zinc with Iron or Steel, of which the following is a specification.

My invention relates to a process of alloying zinc with iron or steel, and also relates to the product of the process as an article of manufacture, and has for its object to mix, combine, infuse, incorporate and alloy zinc with the internal structure 10 of iron or steel objects from their surfaces inward, in whole, or in part to a depth from their surfaces inward sufficient to protect the object from rust and corrosion, and that is also adapted to render the surfaces of the 20 object non-scalable.

I have discovered that any steel or iron object, after having its surfaces thoroughly cleaned of all scale and oily substances by "pickling" in suitable acid solutions and 25 then provided with a coating of zinc by any one of the well known galvanizing processes, may have the metal of the zinc coating absorbed into and mixed, combined and alloyed with the internal structure of the 30 object, in whole or in part, from the surfaces of the object inward, so that the structure and appearance of the coating will be changed, and maintaining the object within such range of heat for an interval of time proportionate to the thickness 35 of the zinc coating and of sufficient duration for the metal of the coating to be substantially all absorbed by the metal of the object.

In practice I obtain the best results by 40 inclosing the coated object in a retort and subjecting it to a heat of about 600° Fahr., for a period of about six hours, according to the thickness of the coating. When 45 cooled and a residuum of dross is cleaned from the surface of the object, the surface will be found covered with a thin semi-transparent grayish blue film of carbonate of zinc, beneath which is formed an alloy 50 of the metal of the iron or steel base with the zinc of the coating to a depth inward from the original surfaces of the iron or steel object of not less than the original thickness of the zinc coating, and generally 55 to a greater depth.

Zinc coated sheets of iron or steel after being treated by my process are made more malleable and are adapted to be bent to form double seams, or beaded, without breaking or scaling, and are converted into 60 a non-corrosive alloy, especially adapting the sheets for roofing, vessels, and all other purposes for which steel or iron plate may be used. Steel or iron sheet metal such as used for the base of tin plates, after being 65 first zinc coated and then converted into an alloy by my process, may be then coated with tin or zinc in the same manner and by the same processes as steel plate is now converted into tin plate and thereby produce 70 non-corrosive tin or galvanized plate. The alloy produced by my process is also adapted to be electro-plated in like manner and by the same processes as ordinarily used. Zinc coated castings, tubing, structural 75 bodies, nails, screws, nuts and bolts and the like, formed of iron or steel, when treated by my process have their outer portion to a depth from the surface inward proportionate to the thickness of the coating 80 alloyed with the zinc of the coating and if free from impurities are made permanently non-corrosive.

The entire body of iron or steel sheet metal, when provided with a coating of 85 zinc of a suitable thickness proportionate to the gage of the sheet, and subjected to my process, will be converted into an alloy of the metal of the coating and the metal of the base sheet which is non-scaling and 90 is also non-rusting provided the base metal is free from impurities which do not alloy with the zinc.

All iron or steel objects after being treated by my process are adapted to receive a high 95 and lasting polish closely resembling in color and quality the polished surface of nickel plated metal.

Any zinc coated iron or steel object, after 100 being converted into an alloy in whole or in part by my process may be afterward heated to redness without dispelling the zinc, which fact makes it practical to first 105 separately provide structural steel or iron, and the rivets by which they are formed into columns and girders, each with a coating of zinc, and after alloying the zinc coating of the several parts therewith by the process described, the parts may be riveted 110 together in the customary way by the al-

loyed rivets to form the columns and girders, which may be riveted together in structural position without lessening the protection of the rivets from corrosion by reason of their having been re-heated and the whole structure in all of its parts will be alike protected from rust and corrosion and made non-scaling.

I am aware that in the process of zinc 10 coating sheet steel known as the sherardizing process, there is produced a slight combination of the surface of the steel plate with the inner portion of the zinc coating thereby produced, and I am also aware that a 15 continuation of the heating forming a part of said sherardizing process will not have the effect to produce the result obtained by my process, as such continuation merely adds to the thickness of the zinc coating without 20 measurably increasing the depth or thickness of the combination of the two metals. My process is therefore wholly separate and distinct from said sherardizing process and in the application of my process to produce 25 the metal alloy aforesaid I do not limit myself to using zinc coated metal in which the coating is produced by that process.

My process and the product thereof is a distinct advance in the art of alloyage and 30 the benefits thereof in the arts it is manifest will be far-reaching in supplying a non-corrosive metal alloy of greater strength than copper and its alloys and at greatly reduced cost.

35 5. What I claim to be new is—

1. The process of alloying zinc with iron or steel, which consists, after providing the surfaces of the body of iron or steel with a coating of zinc, in heating the coated body 40 to a temperature of about 600° Fahrenheit for a period of about six hours and maintaining it about said temperature until the metal of the coating, excepting a residuum of dross, is absorbed by the metal of the 45 body from the original surface of the body inward.

2. The process of mixing, combining and

incorporating zinc with iron or steel, which consists in heating zinc coated iron or steel to a temperature of about 600° Fahrenheit 50 for a time period sufficient to change the appearance and structure of the coating, to wit: a period of about six hours for the thinnest coating and a longer time for thicker coating in proportion to the additional thickness, and then recoating with tin or zinc.

3. The process of mixing, combining and incorporating zinc with iron or steel, which consists in heating zinc coated iron or steel to a temperature of about 600° Fahrenheit 60 for a time period sufficient to change the appearance and structure of the coating, to wit: a period of about six hours for the thinnest coating and a longer time for 65 thicker coating in proportion to the additional thickness.

4. As an article of manufacture the product arising from the subjection of any zinc coated body of iron or steel to a temperature 70 that will change the appearance and structure of the coating, to wit: about 600° Fahrenheit for a time period of about six hours for the thinnest coatings, and a longer time for thicker coatings proportionate to 75 the additional thickness of the coating.

5. As an article of manufacture the product arising from the subjection of any zinc coated body of iron or steel to a temperature 80 that will change the appearance and structure of the coating, to wit: about 600° Fahrenheit for a time period of about six hours for the thinnest coatings, and a longer time for thicker coatings proportionate to 85 the additional thickness of the coating, and then recoated with tin or zinc.

In testimony whereof I have hereunto set my hand at Erie, Pennsylvania, this 16th day of February, 1914, in the presence of two subscribing witnesses.

BENJAMIN F. DIMM.

In presence of—

FRED F. MORAN,  
SAM G. SNELL.